

## UNITED STATES PATENT OFFICE

2,306,899

## ALLOY

Albert J. Phillips, Plainfield, and Albert A. Smith, Jr., Metuchen, N. J., assignors to American Smelting and Refining Company, New York, N. Y., a corporation of New Jersey

No Drawing. Application February 28, 1942,  
Serial No. 432,794

2 Claims. (Cl. 75—167)

This invention relates to lead alloys and more particularly to alloys of lead, calcium and magnesium which, by reason of the properties they possess and exhibit are especially useful wherever a soft ductile material having high resistance to fatigue and creep is desired. The lead alloy products of this invention can be used in the manufacture of such lead products as cable sheathing, roofing and the like where the products must withstand considerable bending and shaping.

The invention in its broadest aspect may be said to provide ternary alloys of lead, calcium and magnesium possessing certain highly beneficial physical properties, and alloys comprising a base alloy of lead, calcium and magnesium with at least one additional alloying constituent imparting further desired properties to the alloy while at the same time retaining or enhancing the beneficial physical properties possessed by the base alloy. This invention is a result of further research and experimentation with related lead alloys, which are the subject of prior patents to Betterton et al. 2,142,835 and 2,142,836 issued January 3, 1939, and wherein it has been discovered unexpectedly that lead containing very small percentage amounts of calcium and magnesium alloyed therewith produce a lead product possessing greatly improved physical properties.

Specifically the invention provides alloys of lead, calcium and magnesium in which the combined calcium and magnesium content amounts to less than 0.02% of the alloy. While 0.002% to 0.009% each of calcium and magnesium is preferred, compositions containing magnesium and calcium within the limits of 0.001% to 0.009%, respectively, can be employed.

Other metals which may be present or added to the lead-magnesium calcium composition are copper, mercury, tin and cadmium, all of which modify the physical properties of the alloy somewhat without adversely affecting the principal physical characteristics of the ternary alloy. Small additions of copper, for instance, may be added to the Ca-Mg lead alloy, to stiffen the alloy. Tin slightly improves its fluidity and casting properties. Bismuth on the order of .02%, as contained in certain commercial leads, may also be present. The amount of modifying or improvement metal which may be incorporated or contained therein should preferably be within the approximate limits of .02% to 3% or as a minimum about three or four times the magnesium content.

The improved properties exhibited by the lead alloys of this invention and which contain relative small percentage amounts of calcium and magnesium as compared with common lead and

antimony-lead alloy is shown in the following table:

|    | Material tested                                                       | Creep at 30° C. on rolled sheet |                                |                                                                     |
|----|-----------------------------------------------------------------------|---------------------------------|--------------------------------|---------------------------------------------------------------------|
|    |                                                                       | Tensile<br>(lbs./sq.<br>in.)    | Percent<br>elongation<br>in 8" | Load in<br>lbs./sq. in.<br>to cause<br>creep of<br>0.1% per<br>year |
| 5  | Common lead                                                           | 1,800                           | 50                             | 150                                                                 |
|    | Alloy containing—<br>0.004% Ca<br>0.004% Mg<br>0.12% Sn<br>Balance Pb | 2,400                           | 50                             | 650                                                                 |
| 15 | Alloy containing—<br>0.009% Ca<br>0.005% Mg<br>0.25% Sn<br>Balance Pb | 2,700                           | 45                             | 800                                                                 |
| 20 | Alloy containing—<br>6.0% Sb<br>Balance Pb                            | 3,800                           | 50                             | 300                                                                 |

The above data clearly show the improvement in creep resistance and tensile strength which is effected by the addition of very small percentage amounts of calcium and magnesium to lead. The calcium-magnesium-lead alloys containing less than 1% tin are decidedly superior in creep resisting properties than that of 6% antimony-lead metal. A lead alloy containing 0.005% magnesium, 0.004% calcium and 0.25% tin is equal to regular 6-8% antimony leads in general corrosion resistance. For cable purposes the use of the calcium-magnesium-lead base metal modified with approx. 0.06% copper or tin and containing about 0.02% bismuth is recommended. Various other metal additions may be made to produce the desired modified product.

The alloy compositions of the present invention may be readily compounded by conventional processes employed by those skilled in the art, as, for example, by simply incorporating the requisite amounts of the alloying constituents in a proper quantity of molten lead. After compounding the new lead alloy it can be used in the manufacture of various articles, for which it is suited, in the conventional manner.

What is claimed is:

1. An alloy consisting of 0.001% to 0.009% calcium, 0.001% to 0.009% magnesium, tin not exceeding 3%, and the balance substantially all lead.
2. An alloy consisting of 0.001% to 0.009% calcium, 0.001% to 0.009% magnesium, 0.01% to 3% tin, copper not exceeding 3% and the balance substantially all lead.

ALBERT J. PHILLIPS.  
ALBERT A. SMITH, JR.